

## UNITED STATES PATENT OFFICE

2,132,557

## METHOD OF TREATING METAL

Samuel H. Bobrov, Gary, Ind., assignor to American Sheet and Tin Plate Company, a corporation of New Jersey

No Drawing. Application April 17, 1936,  
Serial No. 75,017

2 Claims. (Cl. 148--13.1)

This invention relates to a method of treating metals, and more particularly those which are formed into sheets or strip.

In the manufacture of sheets or strip it is necessary to anneal or otherwise heat-treat them in order to impart certain desirable characteristics. According to annealing practice, by way of example, the material is usually placed in a closed vessel and subjected to relatively high temperatures, such as 1000° F. to 1300° F. If sheets form the material to be heat-treated, they are stacked in superimposed relationship; while strip, on the other hand, is coiled. In either case, considerable difficulty is experienced in preventing sticking and discoloration of the material. One method of attempting to obviate this difficulty is to coat the contacting surfaces of the material with a film of hydrocarbon oil. These oils necessarily leave a residue of decomposition which is carbonaceous and combustible. They are therefore only partially effective depending, of course, upon their existence as a uniform film. The following factors greatly affect the film: range of temperature—length of time of exposure to heat—character of gas within the closed vessel—weight, and consequent pressure of sheets or convolutions of coil. It will be readily apparent to those skilled in the art that these factors will widely vary and impair the effectiveness of the film of hydrocarbon oil.

Some mills roughen the surfaces of the sheets, or strip, in order to provide pockets for retaining the film, and thereby obtain better results. However, this operation is costly and is in many instances undesirable to the ultimate consumer.

It is one of the objects of the present invention to eliminate the sticking and discoloration of heat-treated metallic sheets and/or coils.

Another object is to provide a novel inexpensive separating medium which is comparatively indestructible and therefore applicable with equal facility to metals having smooth or roughened surfaces.

A further object is to enable the heat-treatment of sheet or coiled metals by subjecting the same to temperatures which are considerably higher than those heretofore employed.

According to the teachings of the invention, I employ a metallic soap which is dissolved in a suitable organic solvent. The resulting solution, when heated, leaves a separating medium which performs in the manner previously mentioned.

The metallic soap may be prepared by: (A) Agitating together a fatty acid with an aqueous

solution of a water-soluble salt of the required metal, which water soluble salt consists of a compound of the required metal with a weak acid, such as acetic, oxalic, etc. (B) Heating free fatty or resin acids with a suitable metallic compound, usually the oxide, hydroxide or carbonate, and less frequently the acetate, borate, oxalate, or other easily decomposed salt of the required metal. (C) Mixing of aqueous or alcoholic solutions of alkali metal or ammonium soaps with aqueous solutions of the salts of the required metals, whereby a relatively water insoluble metallic soap is precipitated.

The metal thus combined to form a metallic soap may be one of any of the alkaline earth metals, barium, strontium, calcium, magnesium or beryllium. But other metals, not of the alkaline earth group, are also suitable, thus, aluminum, cerium, chromium, cobalt, iron, manganese, nickel, lead, titanium, thorium, zirconium and zinc are also suitable and may be employed for the purpose of this invention. However, the alkali elements, sodium, potassium, lithium, and the ammoniacal radical NH<sub>3</sub> are not suitable to the purpose of applicant's invention and are therefore excluded from consideration.

The metallic soap thus obtained is dissolved in any suitable organic volatile solvent, such as a hydrocarbon oil or oils. Much lighter and more volatile compounds of hydrocarbon may be employed than those heretofore used as a separating medium per se. Complete dissolution of the metallic soap throughout its organic solvent is effected in contradistinction over those compounds which are merely suspended in the solvent. This obviates the necessity of continual mechanical stirring and the tendency of the soaps to precipitate out, whereby the protecting film would eventually be deposited on the metallic articles in globules, or segregated areas.

After a complete dissolution of the metallic soap in its organic solvent, or "carrier", the resulting solution may be stored indefinitely without deleterious effects.

As a specific instance, I have obtained excellent results with 1% magnesium stearate dissolved in light, white-colored 27% Baumé petroleum oil (Saybolt viscosity of 95 to 105 at 100% F.). The percentage of magnesium stearate with respect to the light volatile oil may be varied, depending on the amount of residue which is desired between the material (sheets, or coil). The solution is applied in any suitable manner.

Heretofore, the highest practical annealing

temperature has been around 1300° F., but this can easily be raised another 100° when employing the separating medium of the invention. This higher temperature is very desirable for most materials.

5 The volatilization of the separating medium leaves an indestructible inorganic residue which is not harmful to the smooth bright finish of the material and the sheets or convolutions thereof 10 may be readily separated without sticking or discoloration, which could be attributed to the medium. This residue neither affects the appearance of the material nor hinders its subsequent processing.

15 While I have shown and described several specific embodiments of my invention, it will be understood that I do not wish to be limited exactly thereto, since various modifications may be made without departing from the scope of 20 my invention, as defined by the following claims.

I claim:

1. The method of treating a metallic article which includes coating at least one surface thereof with a solution comprising an organic solvent and a soluble alkaline earth metal soap, and heat-treating said metallic article, to its annealing temperature thereby forming metallic oxides from the originally applied coating through decomposition by heat whereby the sticking of said metallic article to another metallic article is prevented. 5

2. The method of treating a metallic article which includes coating at least one surface thereof with a solution comprising a volatile organic solvent and a soluble alkaline earth metal soap, and heat-treating said metallic article, to its annealing temperature thereby forming metallic oxides from the originally applied coating through decomposition by heat whereby the sticking of said metallic article to another metallic article is prevented. 10 15

SAMUEL H. BOBROV. 20